

June 8, 1943.

H. E. SOMES

2,321,432

METHOD OF QUENCHING HEATED SURFACES

Filed July 7, 1942.



INVENTOR  
Howard E. Somes

BY *John P. Tarbox*  
ATTORNEY

## UNITED STATES PATENT OFFICE

2,321,432

## METHOD OF QUENCHING HEATED SURFACES

Howard E. Somes, Detroit, Mich., assignor to Budd  
Induction Heating, Inc., Philadelphia, Pa., a  
corporation of Michigan

Application July 7, 1942, Serial No. 450,035

2 Claims. (Cl. 148—19.9)

This application is a continuation-in-part of my earlier application Serial No. 250,298, filed January 11, 1939.

This invention relates to a method of quenching heated surfaces for the purpose of hardening them. Although it is particularly adapted to quenching the inner surfaces of cylinders, hub bores and the like, it will be apparent that its use is not limited to any specific type of surface, but that the invention can be employed in quenching substantially any surface configuration.

An object is to provide a method of quenching the heated surface of a workpiece, of such character as to provide an accurate control of the hardening operation so that the pattern of hardness imparted to the surface can be conformed to any predetermined character of uniformity or non-uniformity.

A further object is to provide a method of quenching the heated surface of a workpiece which provides a controllable distribution of the coolant and, if desired, of its hardening effect.

In general, the present invention accomplishes these objects by subjecting substantially the entire area of a heated surface to the simultaneous direct impingement of separate streams of coolant and so regulating the relative volumes and velocities of the different streams as to produce any desired distribution of the coolant over the workpiece. By suitably regulating the volumes and velocities of the separate streams relatively to each other, any predetermined hardening effect can be attained, either a substantially uniformly hardened surface or a surface having different degrees of hardness in different areas, in accord with any predetermined pattern.

The accompanying drawing illustrates one form of apparatus, a quenching head, by which the objects of the present invention can be attained, but it will be apparent that other specific arrangements of apparatus can be employed.

In the drawing:

Figure 1 is a sectional view through one embodiment of a quenching nozzle adapted to be used in carrying out the present method;

Figure 2 is a transverse sectional view on an enlarged scale taken on the line 2—2 of Figure 1; and

Figures 3 and 4 are diagrammatic views showing one spacing of nozzle ports which I have found successful in actual operation.

The particular form of nozzle illustrated comprises a tubular member 10 having a metering pin 12 therein. The nozzle is open at one end

as at 14 and provided with threads 16 for engagement with a coolant supply pipe, not shown. The pin 12 has threads 18 adjacent a head 20 for mounting in and closing the opposite end of the tubular member 10.

The tubular member is provided with a plurality of ports 24, illustrated as arranged in circular rows 26 uniformly spaced along the length of the tubular member. The coolant flows into the open end 14 of the nozzle and is then directed radially outward through the ports, the spacing and arrangement of which are such that, in operation, the entire area of the heated surface is subjected simultaneously to impingement by the coolant, and the ports are so formed that the area of the surface impinged upon by each stream complements and abuts the areas impinged upon by the adjacent streams, as illustrated diagrammatically in Figures 3 and 4. With the ports arranged in this manner the volume and velocity of each stream may be so controlled as to enable accurate control of the hardening action to produce a surface having substantially any predetermined pattern of hardness.

For this purpose the metering pin 12 is formed so as to progressively constrict the bore of the tubular member from the first row of ports adjacent the open end to the ports nearest the closed end. In the illustrated embodiment, the constrictions are produced by successive sections 28 of the pin of progressively increasing diameter, the first section having the smallest diameter being positioned in the bore of the tubular member above the first row of ports 24. Each section 28 of the pin extends from a position opposite one set of ports to a position adjacent the next exceeding row and the successive sections are connected by short conical faces 30. As a result, the cross-sectional area of the annular passage formed by the pin is reduced by a certain amount as indicated at 32, again reduced by a definite amount at 34, again at 36 and so on. By this arrangement the flow of coolant to the various rows of ports can be closely regulated so long as the necessary supply pressure on the coolant is maintained. In order to reduce turbulence within the nozzle and contribute to the flow of large quantities of coolant through the ports, as required in quenching, an annular groove 40 is formed in the member 10 communicating with the ports in each row. Each groove has a sloping entering contour 42 and a curved face 44 tangent to the adjacent walls of the associated ports, and terminating in a ridge 46

so placed as to direct the axial flow of coolant through the member 10 radially into the associated discharge ports 24. As illustrated, each ridge 46 is located adjacent the larger end of the associated conical surface 29.

The present invention is particularly adapted to quenching when the workpiece 50 and the quenching nozzle are relatively stationary during the quenching operation.

In accordance with the present method, coolant flowing into tubular member will have predetermined portions diverted from the main stream at successive discharge ports and the associated parts of the nozzle are so constructed and arranged as to direct streams of coolant upon the heated surface with such relative volumes and velocities as to produce any predetermined hardening effect thereon. For example, the volume and velocity of each stream may be such that the extraction of heat from the entire surface is substantially uniform so as to produce a substantially uniformly hardened surface. On the other hand, control of the streams may be such that the extraction of heat from certain predetermined portions of the heated surface will be slower than from others to produce a variably hardened surface in accordance with any predetermined pattern of hardness. At all times, however, for maximum efficiency, the streams are so controlled and directed that the distance A between the centers of the streams at the heated surface, and their operation is such that the surface area impinged upon by each stream complements and abuts the area impinged upon by the adjacent streams so that every portion of the heated surface is subject to direct impingement by the coolant, as indicated diagrammatically in Figures 3 and 4 in which the workpiece is shown as a portion of an inner cylindrical surface. As shown in Figures 3 and 4, each stream center is equi-distant from the centers of each adjacent stream.

It will be apparent that the present method can be carried out by other forms of apparatus than that illustrated, and that it is capable of being variously modified and adapted within the

scope of the appending claims without departing from the spirit of the invention.

What is claimed is:

1. The method of quenching a heated surface which consists in separating a stream of quenching fluid into a plurality of separate streams, directing said streams against said surface from a distance substantially in excess of that needed for the removal of quenching fluid after its impingement on said surface, directing said streams simultaneously against the surface in such spaced relationship as to cause quenching fluid to impinge directly on substantially all parts of said surface with the center of each stream at the point of impingement substantially equally spaced from the center of each adjacent stream and controlling the quantity and velocity of said streams so that each stream delivers that quantity of quenching fluid per unit of time which equates the extraction of heat per unit of area per unit of time from that surface area upon which a stream impinges with the extraction of heat from each other unit of area upon which the other streams impinge.
2. The method of quenching a heated surface which consists of separating a stream of quenching fluid into a plurality of separate streams, directing said streams against said surface from a distance substantially in excess of that needed for the removal of quenching fluid after its impingement on said surface, directing said stream simultaneously against said surface in such spaced relationship as to cause quenching fluid to impinge directly on substantially all parts of said surface with the center of each stream at the point of impingement substantially equally spaced from the center of each adjacent stream, and controlling the quantity and velocity of said streams so that each stream delivers that quantity of quenching fluid per unit of time which is required to produce in cooperation with the quantity delivered by each other stream substantially uniform extraction of heat per unit of time throughout the area quenched.

HOWARD E. SOMES.